

## UNITED STATES PATENT OFFICE

HAROLD SIMMONS BOOTH, GILBERTA G. TORREY, AND MENAHEM MERLUB-SOBEL, OF CLEVELAND HEIGHTS, OHIO

## METHOD FOR THE ELECTROLYTIC DEPOSITION OF METALS

No Drawing.

Application filed June 26, 1930. Serial No. 464,104.

This invention in one of its aspects, relates to a method for the electrodeposition of certain metals, which cannot be electrodeposited from aqueous solutions, as well as metals, which though it is possible to electrolytically deposit them from aqueous solutions, such method is not satisfactory because it results in low current efficiencies and considerable hydrogen is released at the cathode simultaneously with the deposition of metal, which adversely affects the character of the deposit and results in high commercial cost of operation.

In another aspect of the invention it relates to a method for the electrodeposition of metals other than those in the class prescribed above, wherein the electrolytic deposition is carried on in a solution of an appropriate salt of the metal in liquid ammonia or substituted ammonias (inorganic or organic or a mixture thereof) while maintaining the temperature of the solution above the boiling point of the ammonia, in other words at room temperatures, and raising the boiling point of the ammonia by conducting the electrolytic operation under pressure, or by the addition to the solution of a suitable substance or substances, the effect of which will be to raise the boiling point of the solution.

A still further aspect of the invention relates to the electrodeposition of metals of the class above prescribed, and in addition, other metals outside of the prescribed classes, in which there is dissolved in the liquid ammonia or substituted ammonias (as above referred to), a cyanide compound of the metal which is to be electrolytically deposited, such as cyanides, cyanate and thiocyanate.

We have found that by the use of appropriate salts dissolved in liquid ammonia or substituted ammonias, (inorganic or organic or a mixture thereof) it is possible to obtain electrodeposition of metals, which are not at all obtainable from water solution, and on the other hand, to obtain a more efficient, as well as better deposition of metals, which are capable of electrolytic deposition from water solution. We have found that compact adherent metal deposits are quite feasible from liquid ammonia solution (and its sub-

stituted compound) by the use of proper voltage and current density, both at low temperatures while maintaining the liquid bath under pressure to control the boiling point of the liquid ammonia, or at artificially maintained higher temperatures and under normal pressure conditions.

We have found that metals electrodeposited from solution of ammonia or substituted ammonias, possess unusual corrosion resisting characteristics, probably due to the favorable conditions under which deposition has taken place.

As an example of one application of the present invention, we would refer to the electrodeposition of beryllium, which metal, so far as we are aware, has never before been electrolytically deposited from any solvent, and, so far as we are aware, is obtainable only by the use of fused electrolytes. For example, the iodide of beryllium may be dissolved in ammonia at about the boiling point of the solvent, and upon electrolysis there will be obtained a deposition of beryllium on the cathode. Chloride of beryllium may be used equally well, although with the last named solute, it is preferable to operate while maintaining suitable pressure within the electrolytic cell at normal temperatures. The higher temperature obtainable under pressure, gives the beryllium chloride greater solubility.

While reference has here been made to the use of liquid ammonia, it will be understood that substituted ammonias will also act as a solvent and give the desired deposition of beryllium, (even as complex a substituted unit as piperidine gives positive results). The use of liquid ammonia as a solvent is preferred largely on account of lower cost.

In addition to the use of pressure, in order to raise the boiling point of the liquid ammonia, we have found it feasible to obtain the same effect by the addition of certain salts to the liquid ammonia, as examples of which we may cite ammonium thiocyanate and the like, or certain inert materials which are soluble in liquid ammonia, as an example of which we may mention sugar, which because of their great solubility raise the boiling point

of ammonia, (thus reducing its vapor pressure) and thus making possible electrolytic operation at higher temperatures.

It is quite possible to use the dehydrated forms of other salts, which must be dehydrated because the presence of water of crystallization would interfere with efficient deposition. As an example of such a dehydrated salt we would mention the anhydrous 5 nitrate of beryllium, which can be used for the electrolytic deposition of beryllium, either at the boiling point of ammonia or at room 10 temperatures (as before explained).

Without in any way intending to limit the 15 scope of the present invention, we would give one or two examples of the operation of the foregoing invention.

Anhydrous beryllium iodide may be dissolved in liquid ammonia about six grams of 20 salt to every one hundred cubic centimeters of the solvent at the normal boiling point of ammonia. This solvent is subjected to electrolytic action, using about twelve to fifteen amperes per square decimeter of cathode area. 25 The voltage necessary will vary with the effectiveness of the stirring of the solution, and will also be affected whether or not a beryllium anode is used. The cathodic current density is by no means critical. A very 30 satisfactory deposition of metallic beryllium was thus obtained.

As another example we would state that a 35 satisfactory deposition of beryllium was obtained from a saturated solution of beryllium chloride in liquid ammonia (temperature of the bath approximately  $-38^{\circ}$  C.) using a current density of 2.5 amperes per square decimeter and a line voltage of 10 volts. As 40 illustrating a variation of both current density and voltage, with a solution as above mentioned, a perhaps more satisfactory deposit was obtained by using a current density of 0.6 amperes per square decimeter and a line voltage of 4 volts.

45 As another example of the electrolytic disposition of metals which cannot be deposited from aqueous solutions, we would cite the case of boron. A solution of a halide of boron in liquid ammonia (at either low or high temperatures and pressures) will, upon electrolysis of the solution, deposit metallic boron at the cathode.

50 Manganese may be cited as an example of a class of metals which can be electrolytically deposited to some extent, from aqueous solution, but gives considerable difficulty of one kind or another. Salts of this metal when electrolytically deposited in a water solution, give a small amount of deposition, but the 55 deposit soon deteriorates upon continued electrolytic action. Moreover, there is a great tendency for the metal to oxidize, in the same manner as iron will rust.

55 On the other hand, using manganese salts, as for instance, manganese thiocyanate, dis-

solved in liquid ammonia, either with or without the addition of agents to raise the boiling point of the liquid (as pointed out in the earlier part of this specification), or under pressure, we are able to obtain a very 70 satisfactory deposit of metallic manganese with a very satisfactory current efficiency, and further, we find that the metal is of greater purity and will withstand deterioration in 75 corrosive atmosphere for a long period of time.

As a practical example of the electrolytic deposition of manganese, we would state that 80 good deposition yield has been obtained by using about one gram of manganese thiocyanate for every one hundred cubic centimeters of liquid ammonia (at the boiling point of ammonia). The current density must be regulated to the concentration of the salt, but when the concentration, as given above, is 85 used, a current density of about two-tenths amperes per square decimeter of cathode surface gives good results. If metallic manganese is used as an anode, the corrosion of 90 the above is almost perfect.

95 Chromium is also a metal which can be deposited from liquid ammonia solution, much more satisfactorily than it can be deposited from a solution of chromium salts in water. By the use of chromic thiocyanate (the violet form is preferable over the green form, because of solubility, although the green form turns to the violet form on contact with ammonia) chromium can be deposited upon 100 the cathode electrolytically with far better "throwing power" than any aqueous solutions, with which we are conversant.

105 Since poor "throwing power" is one of the outstanding difficulties in present day chromium plating practice, electrolytic deposition from liquid ammonia solutions presents great advantages over the usual chromium plating practices at present in use.

We would further point out that many 110 metals, though giving relatively high current efficiencies when electrolytically deposited in a water solution, can better be deposited from liquid ammonia solution at temperatures higher than the boiling point, but not at the low temperature of the boiling point of ammonia.

115 We have found that many of the obstacles inherent in low temperature electrolysis, are automatically eliminated in raising the temperature of operation to the normal, either by pressure or by the presence of a material in the solution, the result of which is to raise the boiling point thereof.

120 When using pressure, besides the temperature factor itself, and its corollary increase in the solubility of salts, there is one additional factor of importance to be considered, to-wit, that the increase in pressure acts to 125 prevent the evolution of hydrogen, in the 130

case of those metals higher in the electromotive series than the hydrogen itself.

Without intending any limitation, we would state that we have found that the best 5 deposition occurs where the metal salts used are cyanides or cyanide addition compounds, such as cyanates, thiocyanates and similar compounds.

Where in the claims the word ammonia is 10 used without qualification, we intend that it shall be taken as a generic term, including liquid ammonia as well as substituted ammonia, either inorganic or organic. Also in the claims where the term cyanide compound 15 is used it is intended to be generic, and to include not only cyanides, but cyanide addition compounds, such as cyanate and thiocyanate.

It will be understood that various deviations 20 may be made from the disclosure of the invention heretofore given, without departing from the spirit of the invention, and such deviations are considered to be within the purview of the present invention.

25 Having thus described our invention what we claim is:

1. The method for electrodeposition of beryllium which consists in electrolyzing a solution of a salt of beryllium in ammonia. 30 2. The method for electrodeposition of beryllium which consists in electrolyzing a solution of a salt of beryllium in liquid ammonia. 35 3. The method of electrodeposition of beryllium which consists in electrolyzing a solution of a salt of beryllium in liquid ammonia and adding to the solution ammonia-soluble materials to raise the normal boiling point of the liquid ammonia, the temperature of the solution being above the normal boiling point of the liquid ammonia. 40

45 4. The method of electrodeposition of beryllium which consists in electrolyzing a solution of a salt of beryllium in liquid ammonia, the said solution being maintained under pressure greater than atmosphere and the temperature of the solution being above the normal boiling point of the liquid ammonia.

In testimony whereof, we hereunto affix 50 our signatures.

HAROLD SIMMONS BOOTH.  
GILBERTA G. TORREY  
MENAHEM MERLUB-SOBEL